

## UNITED STATES PATENT OFFICE

2,240,470

## PHOTOGRAPHIC GELATIN LAYER CONTAINING A MONOESTER OF SORBITOL

Donald R. Swan, Rochester, N. Y., assignor to  
Eastman Kodak Company, Rochester, N. Y., a  
corporation of New Jersey

No Drawing. Application March 2, 1940,  
Serial No. 321,901

7 Claims. (Cl. 95—7)

This invention relates to photographic light-sensitive materials, such as sensitized film, plates, and paper, comprising layers in which sensitive silver salts are suspended or dispersed in gelatin or other suitable vehicle, and optionally comprising other layers as well. More particularly, it relates to the use of certain agents to facilitate the spreading of gelatino-silver-halide layers and, in fact, the spreading of any gelatin or other hydrophilic colloid layers which are deposited from a predominantly aqueous medium and used in such photographic materials.

My invention perhaps finds its greatest usefulness in the manufacture of photographic film in which a sensitive gelatin emulsion layer is applied to the film base, set by chilling, and then, without drying, is overcoated with a protective gelatin layer, the sensitive gelatin emulsion layer containing such a spreading agent. The general process of coating film base with a sensitive gelatin emulsion layer, setting by chilling, and overcoating with a protective gelatin layer, is fully set forth in U. S. Patent No. 1,699,349 of William B. Dailey.

If a sensitive gelatino-silver-halide emulsion is coated on a film base (which has usually first been coated with a thin layer or sub-stratum of gelatin or other colloid and dried) without the addition of a suitable spreading agent, difficulty is experienced in that the emulsion will spread unevenly. Moreover, if the emulsion while still in a wet, chilled condition, is overcoated with a protective gelatin coating, air bubbles form between the emulsion layer and the protective layer. Either of these defects, of course, greatly impairs the quality of the photographic film.

It has, therefore, been customary in the art to add certain agents, such, for instance, as saponin, to the sensitive emulsion in order to avoid these defects as far as possible. Saponin has surface-active properties, and not only acts as a spreading agent for gelatin, but by some mechanism not clearly understood, it prevents the formation of air bubbles between the gelatin layers when a wet, chilled gelatin emulsion layer containing the proper concentration of saponin is overcoated with a warm gelatin solution.

However, saponin, being a naturally occurring material of vegetable origin, is of varying quality, and synthetic agents are to be preferred because of their more constant and controlled properties. Because of its varying quality, some batches of saponin may cause an increase in fog or a decrease in sensitivity in the sensitive emulsion, and in some cases may produce little

or no improvement in spreading. This is true whether the saponin be employed in the emulsion layer or in the protective overcoating or other layer.

Other surface-active materials have been tried in place of saponin, but many of them, while they may act to some extent as spreading agents for gelatin, have been found to be entirely ineffective for preventing the formation of air bubbles when a wet, chilled gelatin emulsion containing them is overcoated with a warm gelatin solution, and many of them are objectionable from the standpoint of fogging or desensitizing the emulsion.

I have found a class of surface-active compounds which are not only excellent spreading agents for gelatin and other hydrophilic colloid layers which are deposited from a predominantly aqueous medium and used in photographic films, plates, and paper, but which, when dispersed in layers such as sensitive gelatin emulsions, prevent the formation of air bubbles when the wet, chilled emulsion layer is overcoated with a warm gelatin solution or other hydrophilic colloid of the type which is deposited from a predominantly aqueous medium. These compounds are the monoesters of sorbitol with an acid selected from the group consisting of the aliphatic acids of from 8 to 18 carbon atoms and the alicyclic acids. They may be prepared by the partial esterification of sorbitol in pyridine by the acid chloride, in the manner described in U. S. Patent No. 1,959,930 of Otto Schmidt, Example 2. Individual acid chlorides may be used, such as the chlorides of lauric, myristic, oleic, ricinoleic, naphthenic, abietic or hydroabietic acid, or the chlorides of the mixture of acids obtained from coconut oil may be used. Of the aliphatic acids, lauric acid and the mixture of coconut oil acids are preferred.

These sorbitol monoesters are not sufficiently water-soluble to remain for long in a fluid gelatin or similar emulsion. Therefore, it is necessary to disperse them in the gelatin emulsion by means of some water-soluble dispersing agent, such, for instance, as sodium lauryl B-sulfobutyrate, sodium lauryl sulfonate, sodium B-oleylamidoethyl sulfonate, sodium B-lauramidoethyl sulfate, etc. The mixture of sorbitol monoester and dispersing agent may be incorporated in the sensitive gelatin emulsion at any point in its manufacture such that it will be present during the coating of the emulsion, in the proportion of from 0.001 to 0.002 part of sorbitol monoester and from 0.02 to 0.04 part of the dispersing agent per

100 parts by weight of wet emulsion. This gives a sorbitol monoester content of 0.01% to 0.02% and a content of dispersing agent of 0.2% to 0.4% in the dried emulsion layer. These sorbitol monoesters have no detrimental effect upon the photographic properties of the emulsion, but, on the contrary, improve them. For example, they improve the aging qualities of the emulsion. Photographic films in which the sensitive emulsion contains the above-mentioned proportions of the sorbitol monoesters defined have been found to show higher speed and less fog after prolonged storage at elevated temperatures than ordinary film stored for the same length of time under the same conditions. They are also more readily wet by the developing solution.

It is believed that the property of the spreading agent which prevents the formation of air bubbles when a wet, chilled gelatin emulsion is overcoated with a warm gelatin solution, also tends to prevent the formation of air bubbles, repellent spots, etc., on the surface of a sensitive emulsion containing such a spreading agent, when that emulsion, coated on a film, plate, paper, etc., is immersed in a developer.

As above pointed out, the dispersed sorbitol monoesters defined may be used in any one or more of the colloid layers used to build up a photographic sensitive element upon a base such as film, glass, paper, etc., which layers consist of gelatin or other hydrophilic colloid which is deposited from a predominantly aqueous medium, i. e., a medium used as the solvent for such materials in which water predominates, the remainder of the medium contributing to give a good dispersion of the colloid. If two superposed colloid layers are present, either, neither or both of which may be photographically sensitive, the spreading agent may be used in either layer or in both layers. However, where a wet, chilled light-sensitive gelatin or similar layer is to be overcoated with a warm solution or emulsion of gelatin or similar material, the presence of the spreading agent in the wet, chilled layer is essential for preventing the formation of air bubbles between the layers. Examples of such hydrophilic colloids other than gelatin, which are useful as layers in photographic films, plates, paper, etc., are the water-soluble cellulose derivatives such as well hydrolyzed cellulose acetate (described in U. S. Patent No. 2,110,491 of Salo) and cellulose esters of hydroxy monocarboxylic acids, such as lactic or glycolic, and salts of cellulose esters of dicarboxylic acids, such as phthalic (described in U. S. Patent No. 2,127,573 of Sheppard and U. S. Patent No. 2,127,621 of Staud), as well as polyvinyl alcohol and hydrolyzed polyvinyl acetate (described in applications of Wesley G. Lowe, Serial Nos. 318,559 and 318,560, filed Feb-

ruary 12, 1940) and water-soluble polyvinyl acetals (described in an application of Charles R. Fordyce, Serial No. 221,584, filed July 27, 1938, Patent No. 2,211,323). When colloids other than gelatin are used, it may be desirable to coat them at different temperatures.

In the claims appended hereto, where a "hydrophilic colloid depositable from a predominantly aqueous medium" is referred to, it will be understood to mean any hydrophilic colloid which can be deposited from a medium which is predominantly aqueous, the remainder of the medium being an organic solvent which contributes to the dispersibility of the colloid; examples of such organic solvents for this purpose are acetone, ethyl alcohol, ethylene glycol, monacetin and pyridine.

What I claim as my invention and desire to be secured by Letters Patent of the United States is:

1. Photographic sensitive material comprising a layer of a hydrophilic colloid depositable from a predominantly aqueous medium, said layer containing, in a dispersed state, from 0.01% to 0.02% of a monoester of sorbitol with an acid selected from the group consisting of the aliphatic acids of from 8 to 18 carbon atoms and the alicyclic acids.

2. Photographic sensitive material comprising a gelatin layer containing in a dispersed state from 0.01% to 0.02% of a monoester of sorbitol with an acid selected from the group consisting of the aliphatic acids of from 8 to 18 carbon atoms and the alicyclic acids.

3. Photographic sensitive material comprising a base and two superposed gelatin layers, in which the gelatin layer nearer the base contains, in a dispersed state, from 0.01% to 0.02% of a monoester of sorbitol with an acid selected from the group consisting of the aliphatic acids of from 8 to 18 carbon atoms and the alicyclic acids.

4. Photographic sensitive material comprising a base, a photo-sensitive gelatin emulsion layer and a gelatin overcoating on the emulsion, in which the photo-sensitive gelatin emulsion layer contains, in a dispersed state, from 0.01% to 0.02% of a monoester of sorbitol with an acid selected from the group consisting of the aliphatic acids of from 8 to 18 carbon atoms and the alicyclic acids.

5. Photographic sensitive material comprising a gelatin layer containing, in a dispersed state, from 0.01% to 0.02% of sorbitol monolaurate.

6. Photographic sensitive material comprising a gelatin layer containing, in a dispersed state, from 0.01% to 0.02% of sorbitol mono-naphthenate.

7. Photographic sensitive material comprising a gelatin layer containing, in a dispersed state, from 0.01% to 0.02% of sorbitol mono-hydroabietate.

DONALD R. SWAN.